

(No Model.)

L. SCHNADEL.

PROCESS OF TANNING HIDES.

No. 293,364.

Patented Feb. 12, 1884.



# UNITED STATES PATENT OFFICE.

LOUIS SCHNADEL, OF CHICAGO, ILLINOIS.

## PROCESS OF TANNING HIDES.

SPECIFICATION forming part of Letters Patent No. 293,364, dated February 12, 1884.

Application filed June 23, 1883. (No. model.)

*To all whom it may concern:*

Be it known that I, LOUIS SCHNADEL, a citizen of the United States, residing in Chicago, in the State of Illinois, have invented certain 5 new and useful Improvements in the Process of Tanning Hides, of which the following is a specification.

My object is to lessen the bark used, and produce a better leather in less time, and add 10 more weight to it.

The accompanying drawing shows the internal arrangement of a tannery.

The vats, marked A are leaching-vats; B, layer-vats; C, lime-vats; D, bed-mill; E, color-mill; 15 F, hide-mill; G, receiving-tank for distributing the liquor after being used; H, soaking-vats.

The first operation is to put the hides into fresh water for five or six hours, then into the hide-mill for one-half hour. The hide-mill is 20 a vat having a long wheel with open buckets that, as it revolves, stirs up the hides; then into fresh water—in the summer, thirty-four hours, in the winter, thirty-six hours; then back into the hide-mill one-half hour. After 25 this operation all the superfluous flesh is taken off by the ordinary means. It is then put into the several lime-vats and changed from one to another until the hide has been into five lime-vats. The lime-water in the first vat 30 must be 25° in strength, and the hide remains therein one day. It is then changed into the second vat, the lime-water being 26°, and remains one day. It is then changed into the third vat, the lime-water being 28°, for one 35 day; then into the fourth vat, the lime-water being 32°, for one day; then into the fifth vat, the lime-water being 35°, for one day. If any change is made in these several periods of time, the lime-water must be changed in 40 strength in the same proportion. The hide is then put into a sixth vat of pure water. This is followed up until three several packs have passed through the several vats. By this time a large quantity of lime has been deposited in 45 the fresh-water vat. I then draw out the exhausted lime-water in No. 1 and add to No. 6 one barrel of lime, and fill No. 1 with fresh water, and then follow that up with three more packs of hides in the same manner. By 50 thus going around continuously I make and keep the lime-water of a right degree of

strength, and economize the lime. The water must be kept at 60° in the summer and 80° in the winter. The hide is then washed in the hide-mill until the lime is entirely cleaned off. 55 The hide is then put into the bed, which I make of human excrement of 3° to 4° of strength, or fowl-manure in the following proportions and 4° to 5° of strength: one and one-half bushel to one hundred heavy hides; 60 one bushel to a hundred light sides; three-fourths bushel to one hundred light kips; one-half bushel for two hundred calf.

The bed-mill is similar in construction to the hide-mill—that is, the vat has a revolving 65 wheel in it to agitate the hides. The mill is run five hours and the hide remains in twelve hours after the stoppage of the wheel. The hide is then put into the hide-mill and washed clean in cool water. It is then soaked in tem- 70 perately warm water about one to two hours. Then the fine hair is taken off. It is then put into the color-mill, the liquor of which is made of hemlock or oak bark and water, and must be 4° to 5° of strength. The hide is left in 75 three hours, and stirred by a moving wheel therein or otherwise. Then it is taken out and put into the handling-vats. The operation there is to change it from one to the other until it has passed through six vats, remaining 80 a day in each, the liquor of each one increasing one-fourth of a degree in strength up to the last vat. It is then put into the layer-vats, which consist of a layer of hides and a layer 85 of fine bark in as many layers as required, and changed from one to another until it has been in five successive vats, having the liquor in the following degrees of strength and remaining the following lengths of time: in the first layer-vat three days, liquor 8° to 9°; then into 90 vat No. 2, six days, liquor 10° to 11°; No. 3 vat, nine days, liquor 12° to 13°; No. 4 vat, twelve days, liquor 14° to 15°; No. 5 vat, fifteen days, liquor 17° to 18°. By this process the hide is gradually permeated by the liquor. 95 The liquor of these vats must be especially prepared according to my plan, both to get good liquor and get all the strength out of the bark. The bark is ground into the several leaching-vats, made of wood, and in any desired shape and size, and six or more in number. 100 I use six to a set, so that the process

hereinafter stated makes the entire revolution in one week, all the leaches being filled with bark and liquor except the first or No. 1. I fill No. 1 with fresh-ground bark and pump 5 No. 6 into No. 1, and out of No. 5 into No. 6, out of No. 4 into No. 5, out of No. 3 into No. 4, and out of No. 2 into No. 3. Then No. 2 is 10 filled from the tank which holds the liquor that has been already used in other parts of the tanning process. After the liquor has 15 been run over the vat No. 1 three times and used in the layer-vats and tempered to suit the several layer-vats, as hereinbefore stated, then part of the exhausted liquor of the handling-vats is run into the color-mill, as much as is necessary to fill it. The remainder of the liquor 20 in the handling-vats is run over the same leach No. 1, and, being strengthened and purified, is run back into the handling-vats. I can run weak liquor over this leach from the storage-tank until time for steaming, which comes 25 every six days, when six vats are used. In the meantime leach No. 3, having been treated as No. 1 there will be a small percentage of tannin 30 left in the bark. I now steam it and the residue is passed over into the next vat and goes on with the other liquor, getting cool before being used. This is of the greatest importance, as unless it is cool it spots the hide and 35 rots it. The same process is used in all of the several vats—that is, the bark in No. 2 being treated and exhausted as No. 1 it is thrown out and filled with fresh-ground bark, and while this is being run over by exhausted liquor, as No. 1, No. 4 is ready for steaming, that vat having been treated as No. 1, so that 40 by filling and treating each as above described I keep rotating the leaching and steaming in succession throughout any space of time, and by thus continually using the liquor over and

running it through fresh-ground bark it gains strength and is cleared of impurities deposited in it by hides having been through it. This is the only means by which hides can be treated without a risk of spoiling. By the ordinary 45 process large quantities of hides are lost in the tanneries of the country. Often whole yards are lost by the liquor not being kept pure; whereas I can by the above-mentioned process keep the liquor pure and prevent that 50 loss.

It can easily be seen by the several leachings above stated the liquor as it passes through the fresh bark is filtered and strengthened. By this process I am enabled to make a saving 55 of forty per cent. of the bark, a desirable object, as that article is growing scarce every year. I also make the leather in a shorter space of time and add more weight to a hide, and produce a better article, and prevent any 60 loss in the beam-house, where great loss often takes place.

What I claim, and am desirous of securing by Letters Patent, is—

The process of tanning hides consisting in, 65 first, treating the hides in fresh water and in the hide-mill; second, placing the hides in the lime-vats until the coarser hair is taken off; third, washing the hides; fourth, placing the 70 hides in a bed made of human excrement or fowl-manure; fifth, washing the hides clean; sixth, soaking them in water until the fine-hair is taken off; seventh, placing the hides in a coloring-mill; eighth, then placing them in handling-vats; ninth, placing the hides in 75 the layer-vats, substantially as described.

LOUIS SCHNADEL.

Witnesses:

JAS. LORENZO GAGE,  
LOUIS W. H. NEELY.